

J. S. McGIEHAN.

## PROCESS OF IMPREGNATING FABRICS WITH RUBBER.

APPLICATION FILED DEC. 17, 1915.

1,228,458.

Patented June 5, 1917.

3 SHEETS—SHEET 1.



Witnessed  
J.E. Coleman  
Estelle Adelman

1,228,458.

I. S. McGIEHAN.

PROCESS OF IMPREGNATING FABRICS WITH RUBBER;  
APPLICATION FILED DEC. 17, 1915.

Patented June 5, 1917.

3 SHEETS—SHEET 2.



Witnessed  
J. E. Coleman  
Estelle Adelman

Inventor  
Iraae S. McGiehan

I. S. McGIEHAN.  
 PROCESS OF IMPREGNATING FABRICS WITH RUBBER.  
 APPLICATION FILED DEC. 17, 1915.  
**1,228,458.** Patented June 5, 1917.

3 SHEETS—SHEET 3.



Witnessed  
 J. C. Calenian  
 Estelle Adelman

Inventor  
 Isaac S. McGiehan

# UNITED STATES PATENT OFFICE.

ISAAC S. McGIEHAN, OF NEW YORK, N. Y.

## PROCESS OF IMPREGNATING FABRICS WITH RUBBER.

1,228,458.

Specification of Letters Patent.

Patented June 5, 1917.

Application filed December 17, 1915. Serial No. 67,473.

To all whom it may concern:

Be it known that I, ISAAC SEAMAN McGIEHAN, a citizen of the United States, and residing at New York city, in the county of New York and State of New York, have invented a new and useful Improvement in the Process of Impregnating Fabrics with Rubber, of which the following is a specification.

10 My invention relates to processes for filling and coating fabrics with rubber; and to a new product which results from the performance of the process.

The process involves the flexing or bending of the fibers of the material, whereby the interstices are opened up in order to enable the rubber solution to find access to and impregnate all the parts of the fabric including the hollow tubular portions of the 20 threads.

The process also involves a first or preliminary drying and a second drying of the fabric, performed after impregnation. The final step of the process is the application 25 to the impregnated fibrous materials of a uniform coating, which, after being laid, is forced into the fabric by rolls having yielding surfaces, in order to compact the mass as much as possible and to cause the rubber 30 solution to fill any unoccupied spaces remaining at this stage of the process.

The apparatus consists of several closely associated mechanisms, all of which coöperate in the performance of the aforesaid 35 steps of the method.

The first element of the machine, is the drier, over which the fabric passes prior to submergence in the vat containing the rubber solution.

40 The second element of the machine is the impregnating device, the essential parts of which are a vat for the rubber solution and the co-acting fluted rollers and pinions through which the fabric runs and by means 45 of which it is flexed or bent back and forth, in such a way, as to open up the interstices of the fibers for the reception of the rubber solution.

The third element of the machine, is a 50 drier containing heating coils arranged in juxtaposition to the path of the guided sheet of impregnated fabric.

The fourth element of the machine, is that which coats the impregnated fabric, 55 this part consisting, essentially, of rolls for sustaining and guiding the fabric, a heater and a roller or a rubber scraper, operating

to level and smooth the coating as it is applied to the fabric.

The fifth element of the machine contains 60 compression rollers, the faces of which are covered with soft vulcanized rubber, which act to convey pressure to the rubber lying in the spaces between the fibers without, at the same time, crushing the fibers of 65 the threads at their points of intersection, crushing the fibers being the difficulty experienced when rollers having unyielding faces are employed for the purpose of compressing frictioned or coated fabrics. 70

The several parts of the machine are connected with a common driving means, the object being to attain synchronism in all the movable elements, so that all parts of the fabric will have the same speed and not 75 have any tendency to slip over the surface of the movable elements.

I have found that in handling rubber coated fabrics, frictional or static electricity is often produced in such quantities 80 as to cause ignition of the volatile solvents and the tendency to do this is more pronounced in the coating mechanism than anywhere else. Here the knife or steel scraper, usually employed for leveling the applied 85 rubber coating, becomes so highly charged as to produce sparks which may ignite the as yet un-evaporated solvent that is present in the rubber. By substituting a roller or a rubber scraper, for a steel scraper, and by 90 arranging all movable parts of the machine in such a way as to avoid friction, I produce no statical electricity whatever, and render the manufacture of rubber impregnated and coated fabrics entirely safe. 95

The fabric employed by me is one which contains threads composed of twisted strands and is preferably of the open mesh variety. The object being to afford room within the body of the fabric, that is to say, 100 within its interstices both inside and outside of the threads, for containing a relatively large body of rubber, which is in effect, a continuation of the coating of rubber that is super-imposed upon the body of 105 the fabric. This inclosed part of the rubber being inter-locked with the material portion of the fabric, is securely anchored to the fabric, thereby giving the whole fabrication a strength which it would not otherwise possess. 110

In the accompanying drawings which form a part of this specification, the mechanical part of my invention is fully illus-

trated with similar numbers to indicate corresponding parts as follows:

Figure 1 is a side elevation of my entire machine and Fig. 2 is a plan view thereof.

5 Fig. 3 is a side elevation of the impregnating mechanisms showing the details thereof, and Fig. 4 is a plan view thereof.

Fig. 5 is a side elevation of the coating and the compressing devices and Fig. 6 is a front 10 elevation of the compressing mechanism.

"A" (Fig. 1) is a preliminary drier containing a heating cylinder 1, over which a strip of fabric, as yet unimpregnated and uncoated, runs. This cylinder 1 is driven 15 by the main shaft X of the machine through a worm and gear connection 2 and pulley and a belt connection 3.

The impregnating machine "B" consists of a vat 12, having mounted therein, a fluted 20 roller 13 (Fig. 3) that is driven by a sprocket wheel 14, connected by a pulley and belt connection 15 (Fig. 1) and a worm and gear connection 16, to the driving shaft X.

The pinions or idlers, 17, are driven by the 25 fluted roller 13. The cover of the vat has openings or slits for the passage of the fabric into and out of the machine and between these two slits the fabric extends sinuously between the flutes of the roller 13 and the 30 teeth of the pinions or idlers 17. It will be observed that when the fluted rollers and pinions or idlers are rotating, these sinuous parts of the fabric will be bent back and forth over the respective flutes and teeth, 35 and consequently the interstices will be opened up on opposite sides, thereby admitting the rubber solution which, flowing into and filling the interstices will be able to reach and enter the hollow tubular centers 40 of the threads of the fabric.

This result cannot be obtained by pressure alone, for the viscosity of the rubber solution so impedes its flow, that even under a very great pressure, it will not invade extremely small capillary ducts of the kind found in a rubber coated textile fabric. When however, the fibers are temporarily loosened up so as to increase the size of the interstices, the rubber solution will, by capillary attraction, find access to all parts of the fabric and cohere throughout the mass.

The second drier "C" contains a heating coil 21 and guide rollers 22, over which rollers, the fabric runs in proximity to the heating coil 21.

The coating machine "D" is provided with the usual guide rolls 31 and a heater 32. The coating material is applied at 33. The coating material is applied preferably by 60 hand at the portion of the travel of the fabric marked 33 in the drawings, and for that reason the means for applying the coating material are not illustrated, such means

consisting preferably of the manual application by the hands of an attendant. A 65 roller 34, or a rubber scraper, used as a substitute for the ordinary steel knife or scraper, levels and smooths the newly applied coating of rubber.

The advantages of employing this roller 70 or rubber scraper 34 instead of a steel scraper, is that the roller or rubber scraper, unlike the steel scraper, will not, as heretofore explained, produce static electrical charges. 75

The compressing machine contains two rubber coated rollers 41 (Fig. 5) that are forced toward each other by springs 42, the stiffness of which may be regulated by a hand screw 43. One of these rollers 41, is 80 driven by a worm and gear connection 44 and a belt and pulley connection 45.

51 is a roll of unbleached muslin, which muslin is fed on to a roll 52, that receives the finished rubber filled fabric from the impregnating and coating machine. This muslin operates to keep separated the fresh surfaces of the coated fabric and thus prevent adhesion of those surfaces. 85

Having thus described my invention, what 90 I claim and desire to secure by Letters Patent is:

1. A process of manufacturing rubber coated fabrics consisting in passing the fabric through a rubber solution so as to thoroughly impregnate the fabric with rubber and then applying a coating of rubber to the surface of the fabric, leveling said coating and finally passing the fabric between rollers having yielding surfaces so as to secure density and 100 homogeneity in the product. 95

2. A process of manufacturing rubber coated fabrics consisting in passing the fabric through a rubber solution so as to thoroughly impregnate the fabric with rubber, heating the so impregnated fabric and then applying a coating of rubber to the surface of the same, leveling said coating and finally passing the fabric between rollers having yielding surfaces, substantially as and for 110 the purpose described. 105

3. A process of manufacturing rubber coated fabrics consisting in passing the fabric through a rubber solution so as to thoroughly impregnate the fabric with rubber, then applying a coating of rubber to the surface of the fabric, leveling said coating by flexible scraping means, and finally passing the fabric between rollers having yielding surfaces, so as to secure density and homogeneity. 115 120

ISAAC S. McGIEHAN.

Witnesses:

J. E. COLEMAN,  
E. ADELMAN.